

## UNITED STATES PATENT OFFICE

2,212,130

HEAT TREATMENT OF MAGNESIUM ALLOYS  
CONTAINING ZIRCONIUMFranz Sauerwald, Breslau, Germany, assignor, by  
mesne assignments, to Magnesium Develop-  
ment Corporation, a corporation of DelawareNo Drawing. Application May 12, 1939, Serial  
No. 273,292. In Germany June 4, 1938

6 Claims. (Cl. 148—21.3)

This invention relates to magnesium alloys and covers developments arising out of the invention described in the copending application S. N. 236,-552, of which I am one of the inventors.

In the said copending application there are described magnesium base alloys containing between about 0.05 and 2% of zirconium, which alloys may moreover contain zinc and cadmium either singly or together in amounts which do not

form of a solid solution, to form zirconium hydride which is apparently much less soluble in the magnesium matrix and endeavours to separate out in an extremely finely divided form thereby effecting a hardening of the alloy.

The following table shows how the strength properties of various binary magnesium-zirconium alloys are changed by the heat treatment in an atmosphere of hydrogen.

5

10

15

20

20

| Alloy<br>percent<br>of Zr | Anneal-<br>ing tem-<br>perature,<br>° C. | Anneal-<br>ing time,<br>hours | Tensile<br>strength, kgs.<br>per sq. mm.— |                         | Yield point,<br>kgs. per<br>sq. mm.— |                         | Elongation,<br>percent   |                         |
|---------------------------|------------------------------------------|-------------------------------|-------------------------------------------|-------------------------|--------------------------------------|-------------------------|--------------------------|-------------------------|
|                           |                                          |                               | Before<br>treat-<br>ment                  | After<br>treat-<br>ment | Before<br>treat-<br>ment             | After<br>treat-<br>ment | Before<br>treat-<br>ment | After<br>treat-<br>ment |
| 0.61.....                 | 400                                      | 24                            | 17.3                                      | 19.4                    | 5.4                                  | 8.4                     | 17.0                     | 8.9                     |
| 0.89.....                 | 450                                      | 15                            | 16.5                                      | 20.5                    | 6.6                                  | 11.2                    | 19.5                     | 9.0                     |
| 0.78.....                 | 450                                      | 15                            | 15.0                                      | 18.0                    | 6.2                                  | 8.4                     | 7.0                      | 6.1                     |
| 0.85.....                 | 500                                      | 8                             | 16.3                                      | 17.9                    | 6.0                                  | 8.0                     | 10.0                     | 7.0                     |

substantially exceed the amounts which can be taken up in solid solution.

Exhaustive metallographic researches have revealed that in the high magnesium range of the binary magnesium-zirconium system only a limited amount of zirconium can be taken up in solid solution in magnesium.

At temperatures of about 600° C. magnesium will absorb about 1% of zirconium into solid solution but the solubility of the zirconium decreases considerably as the temperature falls and is only very slight at room temperature. It has also been found that the mechanical strength properties of the binary magnesium-zirconium alloys are not improved to any appreciable extent by heat treatment.

It has now however been ascertained that the mechanical strength properties of the alloys, especially the binary magnesium-zirconium alloys can be considerably increased if such alloys be annealed in the presence of hydrogen at temperatures at which a diffusion of the hydrogen into the alloy takes place. The temperatures necessary for this purpose are in the region of about 300-600° C. and the improved properties of the alloys are apparently due to the fact that the hydrogen diffusing into the alloy combines with the zirconium present in the magnesium in the

It has been further ascertained that in alloys which, in addition to up to 2% of zirconium, contain zinc and cadmium (singly or jointly) up to the limit of saturation for the formation of solid solutions between these last two metals, heat treatment improves the mechanical strength properties of such alloys even in the absence of hydrogen, the yield point, in particular, being very considerably raised in some cases. The elongation slightly decreases but is still sufficient to meet the requirements imposed on cast alloys.

The heat treatment for such ternary or multiple alloys consists in annealing the cast and normally solidified (or also quenched) alloys at temperatures below the boundary line of separation of the zirconium, i. e. at temperatures between about 150 and 400° C. As a rule, a preliminary homogenising heat treatment at temperatures above said boundary line is not only unnecessary, but, if protracted, mostly results in the formation of an extremely coarse crystalline structure. The consequent deterioration of the mechanical properties is so considerable that it cannot be counteracted by the favourable effect of the aforescribed annealing heat treatment.

The following examples show the influence of the aforescribed annealing heat treatment on

25

30

35

40

45

50

the mechanical properties of various alloys containing zirconium.

about 400° C. until the desired improvement has taken place.

| 5  | Alloy   | Annealing   |                 | Tensile strength, kgs. per sq. mm.— |                 | Yield point, kgs. per sq. mm.— |                 | Elongation percent |                 | 5  |
|----|---------|-------------|-----------------|-------------------------------------|-----------------|--------------------------------|-----------------|--------------------|-----------------|----|
|    |         | Temp., ° C. | Duration, hours | Before treatment                    | After treatment | Before treatment               | After treatment | Before treatment   | After treatment |    |
| 10 | 0.7% Zr | 250         | 15              | 19.8                                | 22.0            | 6.8                            | 11.0            | 15.3               | 10.2            | 10 |
|    | 2.0% Zn |             |                 |                                     |                 |                                |                 |                    |                 |    |
| 15 | 0.7% Zr | 250         | 15              | 21.5                                | 24.9            | 9.4                            | 14.2            | 12.8               | 9.2             | 15 |
|    | 2.0% Zn |             |                 |                                     |                 |                                |                 |                    |                 |    |
|    | 2.0% Cd |             |                 |                                     |                 |                                |                 |                    |                 |    |
| 15 | 0.7% Zr | 320         | 24              | 23.7                                | 26.5            | 11.9                           | 16.5            | 12.8               | 8.6             | 20 |
|    | 3.0% Zn |             |                 |                                     |                 |                                |                 |                    |                 |    |
|    | 2.0% Cd |             |                 |                                     |                 |                                |                 |                    |                 |    |
| 20 | 0.7% Zr | 170         | 63              | 26.0                                | 27.1            | 15.4                           | 19.2            | 8.6                | 4.8             | 25 |
|    | 4.0% Zn |             |                 |                                     |                 |                                |                 |                    |                 |    |
|    | 2.0% Cd |             |                 |                                     |                 |                                |                 |                    |                 |    |

20 I claim:

1. A process of improving the strength characteristics of magnesium base alloys containing zirconium in amounts not greater than about 2 per cent, which comprises heating such alloys to 25 temperatures between about 150° C. and about 600° C. until the desired improvement has taken place.

2. A process of improving the strength characteristics of magnesium base alloys containing zirconium in amounts not greater than about 2 per cent, which comprises heating such alloys in 30 the presence of hydrogen to temperatures between about 150° C. and about 600° C. until the desired improvement has taken place.

3. A process of improving the strength characteristics of magnesium base alloys containing zirconium in amounts not greater than about 2 per cent and at least one element of the group 35 consisting of zinc or cadmium in amounts not substantially greater than the solid solubility of the respective elements of said group in magnesium, which comprises heating such alloys to a temperature within the range from about 150 to 40 about 400° C. for at least about 15 hours.

4. A process of improving the strength characteristics of magnesium base alloys containing zirconium in amounts not greater than about 2 per cent and at least one element of the group 25 consisting of zinc or cadmium in amounts not substantially greater than the solid solubility of the respective elements of said group in magnesium, which comprises heating such alloys to a temperature within the range from about 150 to 45 about 400° C. for at least about 15 hours.

5. A process of improving the strength characteristics of binary magnesium zirconium alloys containing not more than about 2 per cent zirconium, which comprises heating such alloys in 50 the presence of hydrogen to a temperature within the range from about 300 to about 600° C. until the desired improvement has taken place.

6. A process of improving the strength characteristics of binary magnesium zirconium alloys containing not more than about 2 per cent zirconium, which comprises heating such alloys in 55 the presence of hydrogen to a temperature of the order of 450° C. for at least about 8 hours.

FRANZ SAUERWALD.